

# UNITED STATES PATENT OFFICE.

JAMES S. SMITH, OF CINCINNATI, OHIO, ASSIGNOR TO HIMSELF AND RICHARD C. GATCH AND PORTER IRON ROOFING COMPANY, BOTH OF SAME PLACE.

## METALLIC PAINT FOR ROOFS, &c.

SPECIFICATION forming part of Letters Patent No. 243,990, dated July 5, 1881.

Application filed April 14, 1881. (No specimens.)

*To all whom it may concern:*

Be it known that I, JAMES S. SMITH, a citizen of the United States, and a resident of Cincinnati, in the county of Hamilton and State 5 of Ohio, have invented certain new and useful Improvements in Metallic Paints for Roofs, &c., of which the following is a specification.

My invention relates to a compound for paints adapted to be used on roofs and metallic surfaces.

It consists in the combination of various ingredients, which will be fully explained in the following specification.

I use the following ingredients, which are 15 preferably combined in the following proportions: Candle-gum, twenty-five pounds, (25;) asphaltum, four hundred and fifty pounds, (450;) resin-pitch, two hundred and seventy-five pounds, (275;) resin-oil, one hundred and 20 thirty-five pounds, (135,) and benzine (deodorized) one hundred and fifteen pounds, (115.)

The parts are usually combined in the following manner: The candle-gum, asphaltum, and resin-pitch are boiled together about one 25 hour and a half and then allowed to cool slowly. When partially cool the resin-oil and benzine are added to reduce the mass to the proper consistency for painting and spreading with a brush. More or less benzine and resin-

oil are added according to the desired consistency.

I have been able to produce a good article by the use of a larger quantity of benzine, dispensing with resin-oil; but the use of both resin-oil and benzine makes a better compound.

I have in some cases used rubber-gum in place of candle-gum, and consider it a substantial equivalent of the same.

A roofing-cement has been composed of coal-tar, clean sand, residuary gum of candles, 40 litharge, water, lime, cement, quicklime, and resin, said ingredients being combined and applied in two separate coats on a roof; but such does not constitute my invention, and is not claimed by me.

What I claim as my invention is—

A compound paint consisting of candle-gum, asphaltum, resin-pitch, resin-oil, and benzine, all combined substantially in the manner and for the purpose set forth.

In testimony whereof I have hereunto set my hand in the presence of two subscribing witnesses.

JAMES S. SMITH.

Witnesses:

JNO. E. JONES,  
J. H. CHARLES SMITH.